

# United States Patent [19]

Bhateja et al.

[11] Patent Number: 4,833,056

[45] Date of Patent: May 23, 1989

[54] MONOCOMPONENT TONER POWDER HAVING STRONG PREFERENCE FOR CHARGING POSITIVELY

[75] Inventors: Sudershan K. Bhateja, Cottage Grove; Chung I. Young, Roseville; Nancy N. Quan, Circle Pines, all of Minn.

[73] Assignee: Minnesota Mining and Manufacturing Company, St. Paul, Minn.

[21] Appl. No.: 155,034

[22] Filed: Feb. 11, 1988

[51] Int. Cl.<sup>4</sup> G03G 9/08; G03G 9/14

[52] U.S. Cl. 430/106.6; 430/110; 430/903

[58] Field of Search 430/110, 903, 106.6

## [56] References Cited

### U.S. PATENT DOCUMENTS

3,816,840 6/1974 Kotz ..... 346/74  
4,189,390 2/1980 Noguchi et al. ..... 430/111  
4,224,396 9/1980 Pollet ..... 430/107  
4,230,787 10/1980 Watanabe et al. ..... 430/107  
4,291,112 9/1981 Lu ..... 430/110  
4,312,933 1/1982 Lu ..... 430/110 X  
4,401,741 3/1983 Miyakawa et al. ..... 430/110  
4,430,408 2/1984 Sitaramiah ..... 430/106.6

4,485,163 11/1984 Miyakawa ..... 430/122  
4,656,111 4/1987 Wakamiya et al. ..... 430/110 X  
4,734,350 3/1988 Lin et al. ..... 430/110

### FOREIGN PATENT DOCUMENTS

59-124342 7/1984 Japan ..... 430/110

### OTHER PUBLICATIONS

Schaffert, R. M., "Electrophotography", Focal/Hastings House, New York, 1985.

Kotz, A. R. and Spreng, R. C., "Electronic Imaging with Monocomponent Toners", The Third Annual Guide to Ribbons and Toners38 , Datek Publishing Company, Newtonville, Mass., Jun., 1982.

Primary Examiner—Paul R. Michl

Assistant Examiner—Jeffrey A. Lindeman

Attorney, Agent, or Firm—Donald M. Sell; Walter N. Kirn; James V. Lilly

[57]

### ABSTRACT

A triboelectrically chargeable monocomponent toner powder is provided which comprises as a binder a mixture of a copolymer of styrene and an acrylate with an amine-containing aliphatic wax as a charge-control agent. The toner is inherently strongly chargeable positively through triboelectric forces.

10 Claims, 2 Drawing Sheets





FIG. 1



FIG. 2



FIG. 3



FIG. 4



FIG. 5

MONOCOMPONENT TONER POWDER HAVING  
STRONG PREFERENCE FOR CHARGING  
POSITIVELY

FIELD OF THE INVENTION

The invention concerns monocomponent (or one-part) toner powder useful in electrophotographic copying non-impact printing processes. More particularly, it relates to dry heat-fusible and pressure-fixable toner powder made of a thermoplastic binder and magnetically responsive material such as magnetite.

DESCRIPTION OF THE RELATED ART

In electrophotographic or xerographic copying or non-impact printing processes, reversal imaging is often preferred over forward imaging for a number of reasons. For example, in forward imaging the entire background area is illuminated. This results in stripes or lines in the background and causes a great deal of scattered light which tends to make the images fuzzy. These problems are overcome through the use of reversal imaging. In this type of imaging only the characters, i.e., the light-struck, uncharged area are illuminated and toned. This is a faster and more energy-efficient imaging because the image area is generally smaller than the background or unimaged area.

Two-component toners tend to be highly effective in reversal imaging in terms of high image density and good contrast due to efficient and controlled triboelectrification (contact electrification) of the numerous, small toner particles through a large surface area of contact with the carrier particles. (See, R. M. Schaffert, "Electrophotography", Focal/Hastings House, New York, 1985 for further details on electrophotography, reversal imaging and triboelectrification).

Monocomponent toners (also referred to herein as one part toners) have not previously provided high image densities and good contrast except at low development speeds. Due to the absence of carrier particles, triboelectrification usually occurs only due to surface contact of the toner with itself or surface contact of the toner with the development roller or the doctor blade. Because of this small surface area of contact, prior monocomponent toners tend to charge primarily by the induction process, i.e., only under an applied electric field. Thus, prior monocomponent toners have been little used for reversal imaging in spite of the fact that monocomponent toner powders offer a number of important advantages over 2-component toners. Some of those advantages have been taught in A. R. Kotz and R. C. Spreng, "Electronic Imaging with Monocomponent Toners" in "The 3rd Annual Guide to Ribbons and Toners", Datek Publishing Company, Newtonville, MA June 1982 and in Wilson U.S. Pat. No. 2,846,333 which describes the use of a magnetic brush system for developing latent images that can be transferred electrostatically and fused onto plain paper. Pollet U.S. Pat. No. 4,224,396 reports that the electrical conductivity of Wilson's toner inhibited electrostatic transfer and uses a quaternary ammonium polymer as a charge control agent to provide toner powders of low resistivity. Pollet's toners may be either monocomponent or used with a carrier.

A number of other monocomponent toner powders have been patented, most of which are chemically similar to that of Pollet, e.g., being formed from a mixture of magnetically responsive material, a thermoplastic

binder such as a copolymer of styrene and an acrylate or a methacrylate, plus additional material, mostly dyes which acts as a charge control agent. See, for example, Watanabe et al. U.S. Pat. No. 4,230,787 where, because the electrical conductivity of a prior toner powder had interfered with transferring it onto paper, an electric charge controlling dyestuff was incorporated into monocomponent toner powder.

Miyakawa et al. U.S. Pat. No. 4,401,741 concerns a monocomponent toner powder which incorporates both a positive charge control agent and a negative charge control agent. Doing so is said to solve problems of flowability and cohesion experienced in the use of prior toner powders.

Miyakawa U.S. Pat. No. 4,485,163 is especially concerned with image sharpness when using a monocomponent toner powder for developing positively charged images on plain paper. Miyakawa says this requires "a certain balance between the magnetic characteristic and charging characteristics at the developing step" (col. 3, lines 42-51), answering this by incorporating into the powder an aliphatic carboxylic acid having at least 14, preferably at least 18, carbon atoms or a metal salt thereof. Miyakawa says that the acid or its salt "has a function to facilitate uniform dispersion of the magnetic material in the finely divided state and is effective for controlling charges of the developer (toner) particles to the negative side" (col. 5, lines 34-40).

Sitaramiah U.S. Pat. No. 4,430,408 discloses a monocomponent toner powder which is said to be less sensitive to changes in the size of the development gap and the doctor blade gap in magnetic brush systems, particularly in recording processes such as have been described in Nelson U.S. Pat. No. 4,121,931, Kotz U.S. Pat. No. 3,816,840 or Kotz U.S. Pat. No. 3,909,258. Sitaramiah accomplishes this by including in the toner powder a fluorine-modified alkyl siloxane and by attaching carbon black to the surface of the particles. Useful thermoplastic binders of the Sitaramiah patent include blends of wax component and a thermoplastic organic resin such as copolymers of styrene and one or more acrylate or methacrylate monomers. Useful wax components include aliphatic waxes such as amide hydroxy waxes, four of which are named at col. 4, lines 55-64.

Like Sitaramiah, most toner powders now on the market contain carbon black, sometimes embedded, sometimes at the surface, and sometimes both embedded and at the surface as in Noguchi et al. U.S. Pat. No. 4,189,390. While one function for the carbon black is to obtain an opaque image, Noguchi uses electrically conductive carbon black for its electrical properties, his toner powder being in the form of "essentially spherical members consisting essentially of plastics binder, magnetic particles and first electrically conductive particles dispersed therein, and second electrically conductive particles embedded on the spherical surface of the member" (col. 2, lines 7-15). Both the first and second electrically conductive particles could be carbon black.

SUMMARY OF THE INVENTION

The invention concerns a monocomponent toner powder which is highly triboelectric in nature in a surprisingly controlled fashion and yields extremely dense images at extraordinarily high speeds. In a preferred case, the resulting images are substantially better fixed

to plain paper than are images obtained with commercially successful monocomponent toner powders.

Images formed with the novel monocomponent toner powder are as good in contrast as heretofore could be achieved by using 2-component toners while avoiding the shortcomings of 2-component toners. The monocomponent toner powder of the invention is also extraordinarily tolerant of variations in copying and non-impact printing processes, including variations in fusing temperatures and the sizes of the development gap. The novel toner powder has a range of desirable fusing temperature and is preferably also forgiving of environmental changes such as changes in relative humidity.

While leading monocomponent toner powders now on the market do not become significantly electrostatically charged until exposed to an electrical potential, as in an inductive process, the novel toner powder is intrinsically triboelectric. Thus, it becomes charged positively merely upon coming in contact with the metallic development roller and the charging tendency is substantially enhanced due to the agitation experienced by the toner powder on the development roller. The presence of a surprisingly large and unexpectedly well-controlled inherent triboelectric charge on the monocomponent is believed to permit imaging at extraordinarily high speeds. Also, the strong preference of the novel toner to charge positively fills another commercial need. While it can be used for forward imaging with negatively-charging photoconductors, most common commercial photoconductors, such as selenium or arsenic triselenide, used for non-impact printing or copying tend to be positively-charging. As such, the novel toner powder can be effectively used for reversal imaging (providing many advantages of reversal imaging discussed above) in many commercial non-impact printers.

Since the novel toner powder gives high image densities at relatively low photoconductor voltages, it can substantially enhance the photoconductor life, which can be a significant advantage as well.

In accordance with the present invention there is provided a monocomponent toner powder which comprises a plurality of discrete particles, each of which comprises a mixture of magnetically responsive material and a thermoplastic binder. The thermoplastic binder comprises a mixture of (a) one or more copolymers of styrene with at least one acrylate or methacrylate monomer, and (b) from 0.5 to 20% by weight of an amine-containing aliphatic wax which acts as a charge control agent. Although other thermoplastic resins can be used in combination with the styreneacrylate copolymer, the latter constitutes a major proportion of any such combination.

#### BRIEF DESCRIPTION OF THE DRAWINGS

In the drawing:

FIG. 1 shows the transmission (optical) density of the developed toner layer versus the applied surface potential at two different development speeds for the triboelectric monocomponent toner powder of the present invention and a prior art toner.

FIG. 2 shows the optical transmission density of the developed toner layer versus the applied surface potential at varying development gaps for the toner powders used to generate the data for FIG. 1.

FIG. 3 is a bar graph showing the comparative fusing quality in terms of resistance to rub-off of prints made

from the toner powders of the invention and the prior art toner.

FIG. 4 is a bar graph showing the comparative fusing quality in terms of resistance to rub-off of prints like those tested in FIG. 3 except being gray instead of black, the toner powders being the same as those used to obtain FIG. 3; and

FIG. 5 is a bar graph showing the comparative fusing quality in terms of the level of adhesion at the toner-paper interface, i.e., in terms of the resistance of the fused toner layer to being removed by pressure-sensitive adhesive tape, the tested toner powders being the same as those used to obtain FIG. 33.

#### DETAILED DESCRIPTION

The styrene-containing copolymer should have a glass-transition temperature ( $T_g$ ) from 45° to 75° C. At a  $T_g$  above 75° C., the novel monocomponent toner powder might not flow, adhere to paper, or fuse well enough at acceptably low fusing temperatures, while at a  $T_g$  below 45° C., the toner powder might not be sufficiently free flowing and might cause blocking under some environmental conditions. Any combination of styrene and at least one of acrylate and methacrylate monomers which provides a  $T_g$  within that preferred range should provide a useful copolymer.

The acrylate and methacrylate monomers useful in the invention preferably are selected from lower alkyl acrylates and methacrylates wherein the alkyl group contains from 1 to 12 carbon atoms. These alkyl groups may be straight or branched chain groups.

Examples of styrene-containing copolymers useful in the invention include the Ionac TM series of materials commercially available from Sybron Chemicals. Specific examples of these materials include Ionac TM X-211 which is understood to be a copolymer of 58 parts styrene and 42 parts methylmethacrylate; Ionac TM X-231 which is understood to be a copolymer of 65 parts styrene and 35 parts n-butylmethacrylate. Another useful styrene-containing monomer comprises the copolymer of 75 to 90 parts styrene and 25 to 100 parts isoctylacrylate. Such copolymers may be made by techniques known in the art such as are described in *Polymerization Processes*, Edited by C. E. Schildknecht and I. Skeist, John Wiley and Sons, Inc., 1977.

The amine-containing aliphatic wax should have a hydrocarbon chain of at least 12 carbon atoms. Otherwise it might unduly soften the thermoplastic binder. Preferably the chain has at least 18 carbon atoms. A preferred amine-containing aliphatic wax which is commercially available is a C<sub>18</sub> aliphatic wax having a secondary amine group, namely, "Armeen" 2HT from the Armac Company, and understood to have the formula (C<sub>18</sub>H)<sub>2</sub>NH. The amine-containing aliphatic wax can be adducted with an acrylate such as fluoro-octyl-sulfonyl-ethyl acrylate or isoctyl acrylate. While the amine-termination of the aliphatic wax preferably is a secondary amine, tertiary and primary amine termination should also be useful.

Preferably the amine-containing aliphatic wax comprises from 1 to 10 percent by weight of the novel toner powder. Concentrations below about 1% might result in a toner having relatively poor charging, while concentrations above about 10% might result in a toner which is too soft. About 2-5% of the amine-containing wax is preferred.

The novel toner powder contains a magnetically responsive material, preferably from 30 to 70% by

weight, in order to facilitate the development of the toner powder on to the photoconductor drum under an electric field and its subsequent transfer on to paper.

The novel toner powder also preferably includes non-conductive (resistively  $>10^{12}$  ohm-cm, preferably about  $10^{15}$  ohm-cm) carbon black when black images are desired. As in the prior art, the carbon black may be dispersed throughout the toner particles, embedded at the surface of the particles or both dispersed throughout and embedded at the surface. In order not to interfere with the triboelectric charging, any carbon black at the surface should be electrically nonconductive, i.e., have a resistivity of more than 10 ohm-cm, preferably about  $10^{15}$  ohm-cm.

The toner powder of the invention may also contain other materials that are commonly used in the art, e.g., hydrophobic silica to facilitate flow.

The following examples illustrate the preparation of preferred triboelectric monocomponent toner powders of the invention. In the examples, all parts are by weight.

#### EXAMPLE 1

|                                                                                                                             |          |
|-----------------------------------------------------------------------------------------------------------------------------|----------|
| Magnetite powder (Citco)                                                                                                    | 60 parts |
| Copolymer of 58 parts of styrene and 42 parts <i>n</i> -butylmethacrylate (Ionac <sup>TM</sup> X-211 from Sybron Chemicals) | 36       |
| Amine-containing aliphatic wax (Armeen <sup>TM</sup> 2HT)                                                                   | 4        |
| Resistive carbon black powder (Raven <sup>TM</sup> 5750 from Columbia Chemicals)                                            | 2        |

The aliphatic wax, which is understood to have the formula  $(C_{18}H_{37})NH$ , was melt-blended into part of the copolymeric base resin, and the blend was hammer-milled to produce a dry blend that passed 20-mesh screen. The remaining base resin was dry-blended with the magnetite and the carbon black powder in a twin-shell blender at room temperature for 2 hours. These two dry blends were mixed in a 30-mm twin-screw co-rotating melt-mixer with the heaters set at temperatures in the range of 120°–150° C. The mixture was flaked on a nipping chill roll directly from the melt mixer. The flakes were hammer-milled to pass 20-mesh screen and then ground to micrometer dimensions in an air-jet mill. The resulting powder was air-classified to particle sizes from 8 to 20 micrometers. To improve the flow characteristics, the powder of the invention was surface-blended with 0.1 weight percent of hydrophobic silica powder ("Aerosil" R-972) for 1 hour at room temperature in a twin shell blender.

#### EXAMPLE 2

|                                              |          |
|----------------------------------------------|----------|
| Magnetite powder (Citco)                     | 60 parts |
| "Ionac" X-211                                | 36       |
| Amine-containing aliphatic wax adduct        | 4        |
| Resistive carbon black powder ("Raven" 5750) | 2        |

The amine-containing aliphatic wax adduct was made using a 1-liter, 3-neck flask equipped with heating mantle, mechanical stirrer, and thermometer. Weighed into the flask were 260 g of the amine-containing aliphatic wax of Example 1 and 300 g of a fluoro-octyl-sulfonyl-ethyl acrylate. Upon heating to 60° C., the mixture

became stirrable. Additional heating to 120° C. while stirring resulted in a completely melted and clear mixture. This was allowed to react at 120–130° C. for 30 minutes, cooled to 110° C., and then poured into a pan where it cooled to a hard, brittle solid at room temperature.

#### Reaction:



This adduct was used in the same way as was the aliphatic wax of Example 1 to make a monocomponent toner powder of the invention.

#### TESTING

Data used to make FIGS. 1 and 2 of the drawing were obtained using the experimental test rig of FIG. 1 of Bhateja et al., "On the Development Behavior of Resistive Monocomponent Toners", *Image Technology, 1985/SPSE 38th Annual Conference* published by Society of Photographic Scientists and Engineers, Springfield, VA, pages 175–179. Data shown in FIGS. 3–5 of the drawing refer to the fusing or fixing quality, i.e., how well the toner powder particles in the imaged area are fused to each other or to the paper surface. These data were obtained by first generating the needed unfused images on plain paper using the novel monocomponent toners of the present invention and a 3M "Secretary" III copying machine operating in the reversal imaging mode (but with its normal heat-fuser disabled). In order to obtain some information about the useful fusing temperature window exhibited by the different toners, the above unfused images were then fused in a versatile test rig by varying only the fusing temperature over a wide range (130°–220°), keeping everything else constant. A silicone hot fuser roll was employed for generating all the fused images for the present work. The fusing test rig employed has been described in A. C. Button and R. C. Edberg, "Hot roll fusing of monocomponent toners", *The 2nd International Congress on Advances in Non-Impact Printing Technologies*, Arlington, VA, Nov. 4–8, 1984, p. 202.

The fusing quality was then evaluated by two different tests: (a) The Crockmeter Test, which is a ruboff or abrasion test and, (b) The Tape-Adhesion Test which measures the levels of adhesion at the toner-paper interface.

The "Crockmeter Test" involves mounting a fresh white piece of cotton fabric on the underside of the plastic plug which is effectively under a constant load, resting it on the image/print to be tested and abrading the image by running the Crockmeter for five cycles.

The McBeth reflectance density of the Crockmeter-tested patches of cloth is a measure of the toner abraded away from the image and is referred to as the Crockmeter Number (CN). Thus, the lower the value of CN, the better the fusing quality. Further details on the Crockmeter test can be found in the following references:

1. S. K. Bhateja and J. R. Gilbert, *Journal of Imaging Technology*, II, 271 (1985)
2. S. K. Bhateja and J. R. Gilbert, *Journal of Imaging*

Technology, II, 278 (1985) 3. S. B. Collins, A. C. Button and R.H. Helland, "Fusing of Single-Component Toners", 4th International Conference on Electrophotography, Washington, D.C., Nov. 1981, p. 179

The tape-adhesion test, described in detail in references 2 and 3 above, involves laying a Scotch brand tape (#810) onto the image to be tested under uniform pressure and peeling it off the image at 180° at a constant speed. The reflectance density of the tested images is a measure of the level of adhesion at the toner-paper interface; the higher numbers indicate better fixing. The units reported are optical density units (O.D.U.).

Used as a "control" in the testing was a commercially available monocomponent toner which is believed to yield prints at least equal in overall image quality to that of those obtained from any other monocomponent toner powder now on the market for use in a "Secretary" III copier. It is below called "Prior Powder A".

In FIG. 1, transmission image densities were measured from images made using the toner powders of Example 1 and 2 in comparison to Prior Powder A at each of the two different development speeds, namely, at 24 cm/sec and 160 cm/sec. Many commercial copiers and non-impact printers operate at about 20-30 cm/sec, but the data of FIG. 1 with toner powders of Examples 1 and 2 demonstrate feasibility of operation at development speeds as high as 160 cm/sec.

In FIG. 1;

Curves 10 and 11 indicate transmission densities at development speeds of 24 and 160 cm/sec., respectively;

Curves 13 and 14 indicate transmission densities attained using the toner powder of Example 2, at development speeds of 24 and 160 cm/sec., respectively, and except that curves 11, 13 and 14 are not shown at the right side of FIG. 1, because their right-side portions substantially duplicate that of curve 10. Curves 16 and 17 indicate transmission densities attained using Prior Powder A at development speeds of 24 and 160 cm/sec., respectively.

It can be seen from FIG. 1 that the toner powders of the invention inherently charge strongly positively due to some triboelectric mechanism, i.e., due to contact with the metallic development roller. By comparison, the Prior Powder A tends to be neutral, i.e., it has no preference for charging positively or negatively (see FIG. 1). This is typical of the monocomponent toners of the prior art which, therefore, tend to operate by the induction process, i.e., they tend to charge only when under an electric potential. But, surprisingly the monocomponent toner powders of the invention exhibit a large and well-controlled inherent charge, despite the small surface area of contact that monocomponent toners typically have with the development roller. The strong preference of the toner powder of the invention to charge positively and the accompanying high image densities make them very attractive for reversal imaging in non-impact printers that utilize a positive charging photoconductor (such as selenium). And, most of the positive photoconductors employed in commercial non-impact printers are positively charging.

It can also be seen from FIG. 1 that at a development speed of 24 cm/sec—a speed currently employed in some commercial copiers—exceedingly dense images can be obtained using each of the toner powders of Examples 1 and 2. Table I shows the ratio  $\alpha$  of the transmission density of the developed toner layer using

toner powder of either Example 1 or Example 2 to the transmission density of the developed toner layer obtained using the Prior Powder A, at varying development voltages and each of the two development speeds chosen for illustration. It can be seen that the ratio  $\alpha$  varies anywhere from 2.09 to  $>10$ , depending upon the development voltage and the development speed. FIG. 1, curves 11 and 14, shows that at a development speed just a little slower than 160 cm/sec, each of the monocomponent toners of Examples 1 and 2 would provide images substantially equal in transmission density to those obtained at only 24 cm/sec using Prior Powder A (Curve 16). This offers a major advantage for the toner powders of the invention over the Prior Powder A (or the prior art) because they will permit operation at the commercially attractive high speeds. The toner powders of the invention offer another major advantage in terms of enhanced photoconductor life. In view of the extremely dense images obtained with the toner powders of the invention, they will permit operation at relatively low photoconductor voltages resulting in much enhanced photoconductor life.

TABLE I

| Development Voltage (V) | Ratio $\alpha$      |      |            |           |
|-------------------------|---------------------|------|------------|-----------|
|                         | 24 cm/sec           |      | 160 cm/sec |           |
|                         | for toner powder of |      | Example 1  | Example 2 |
| -1,300                  | 4.43                | 2.87 | 2.09       | 2.34      |
| -1,000                  | 2.53                | 2.70 | 2.39       | 2.74      |
| -750                    | 2.37                | 2.29 | 5.71       | 7.0       |
| -500                    | 2.97                | 2.97 | 7.5        | 7.0       |
| -200                    | 10.0                | 9.50 | $>10$      | $>10$     |

In FIG. 2, Curves 20, 21 and 22 show transmission densities of images obtained at various voltages using the toner powder of Example 1 at a development speed of 24 cm/sec and development gaps of 0.25, 0.75 and 1.5 mm, respectively. Curves 24, 25 and 26, show transmission densities of images obtained using Prior Powder A under the same conditions, also at development gaps of 0.25, 0.75 and 1.5 mm, respectively. Curves 21 and 22 are not shown at the right side of FIG. 2 because at all positive voltages the image densities are very low (less than 0.2 O.D.U.) and so that the other curves can be seen more clearly. As has been pointed out, the toners of the invention charge strongly positively.

Curve 21 in comparison to curve 24 shows the extraordinary tolerance of the toner powder of Example 1 to large development gap variations. It is surprising that even at a development gap three times as large as that used with the Prior Powder A to obtain curve 24, the toner powder of the invention would provide denser images. This means that using the toner powders of the invention, the development gap will not have to be set or controlled very closely. This kind of gap or machine latitude is extremely desirable in non-impact printing or copying machines.

FIGS. 3 to 5 demonstrate the tolerance of images made on plain paper using the tested toner powders to fusing temperature variations which inevitably occur in non-impact printers and copiers.

In FIG. 3, bars 30, 31 and 32 show the resistance to rub-off, as measured by the Crockmeter Test, of black images made at varying fusing temperatures using the toner powders of Example 1, Example 2, and Prior Powder A, respectively.

In FIG. 4, bars 40, 41 and 42 show the resistance to rub-off, as measured by the Crockmeter Test, of grey images made at varying fusing temperatures using the toner powders of Example 1, Example 2 and Prior Powder A, respectively.

In FIGS. 3 and 4, the various different areas on the bars indicated as a, b, c, d and e represent the following: Areas a=hot offset, i.e., some toner adheres to the Silicone fuser roll which subsequently shows up as a ghost-image on the next print

Areas b=excellent fusing quality, i.e., CN<0.20 O.D.U.

Areas c=good fusing quality, i.e., CN=0.20-0.30 O.D.U.

Areas d=fair fusing quality, i.e., CN=0.30-0.40 15 O.D.U.

Areas e=poor fusing quality, i.e., CN>0.40 O.D.U.

In FIG. 5, bars 50, 51, and 52 show the level of toner-paper adhesion, as measured by the tape test O.D.U., of black images made at varying fusing temperatures using the toner powders of Example 1, Example 2 and Prior Powder A, respectively. The various different areas on the three bars indicate:

Areas a'=hot offset

Areas b'=excellent fusing quality (tape test O.D.U. 25 >1.0)

Areas c'=good fusing quality (tape test O.D.U.=0.-40-1.0)

Areas d'=poor fusing quality (tape test O.D.U. <0.40)

As can be seen from FIGS. 3, 4 and 5, toner powders 30 of Examples 1 and 2 are "compatible" with the silicone fuser rollers over a desirable and a wide range of fusing temperatures, i.e., over a wide temperature range during the fusing process, no toner particles from the imaged area transfer on to, and adhere to, the fuser roll; compatibility with the fuser roll is a feature that a toner must exhibit to be usable, otherwise ghost images can appear on subsequent prints. Comparing FIGS. 3, 4 and 5, it becomes clear that toner powders of Examples 1 35 and 2 provide a much wider fusing temperature window than does Prior Powder A, considering the rub-off resistance in black and grey prints (FIGS. 3 and 4) as well as the toner-paper bond (FIG. 5). In fact, toner powder of Example 1 provides an exceptionally broad 40 fusing temperature window. Fusing temperature, thus, adds another parameter to the forgiving nature of the toner powders of the invention pointed out earlier, for instance, in terms of tolerance to the variations of the development gap, development speed or photoconductor 45 voltage. Such an extreme tolerance on the part of a toner powder in setting the machine parameters, i.e., a wide machine latitude offers a major advantage in terms of its commercial use or applications.

### EXAMPLE 3

The toner powder of this Example was made in the same way as that of Example 2 except that the starting ingredients were as follows:

|                                              |          |
|----------------------------------------------|----------|
| Magnetite powder (Citco)                     | 60 parts |
| "Ionac" X-231                                | 36       |
| Amine-containing aliphatic wax adduct        | 4        |
| Resistive carbon black powder ("Raven" 5750) | 2        |

"Ionac TM X-231 is understood to be a copolymer of 5 parts of styrene and 35 parts of n-butylmethacrylate.

The above adduct was made from 521 parts of (C<sub>18</sub>H<sub>37</sub>):NH and 186 parts of isoctyl acrylate by the same procedure as in Example 2.

The resulting toner powder was tested for transmission image density in the same manner as were the toners of Examples 1 and 2. The doctor blade gap was 0.46mm, the development gap was 0.5mm, and the developer shell rotated at 350rpm (development speed of 24 cm/sec). The transmission densities obtained are set 10 out in Table II.

TABLE II

| Voltage | Transmission Density (O.D.U.) |
|---------|-------------------------------|
| -1300   | 1.12                          |
| -1000   | 0.78                          |
| -850    | 0.49                          |
| -700    | 0.38                          |
| -200    | —                             |
| 200     | 0.03                          |
| 500     | 0.04                          |
| 800     | 0.04                          |
| 1000    | 0.06                          |
| 1300    | 0.27                          |

The data indicate that the toner charged inherently strongly positive.

### EXAMPLE 4

A styrene-isoctyl acrylate copolymer was made using a 2-liter split flask equipped with an agitator, a condenser; a nitrogen purge and a temperature control. Weighed into the flask were 8g Ca<sub>3</sub>(PO<sub>4</sub>)<sub>2</sub>, 0.1 g of 1% by weight sodium lauryl sulfate in water, and 800g of deionized water. The ingredients were heated to 70° C. with agitation under a nitrogen purge until all of the Ca<sub>3</sub>(PO<sub>4</sub>)<sub>2</sub>, was dispersed. A premix consisting of 350g of styrene, 50g of isoctylacrylate, 0.1 g of isoctyl thioglycolate and 2g of AZO-bis-isobutyronitrile was prepared and then added to the flask. The temperature control was set to 70° C. and the ingredients allowed to react for 16 hours under nitrogen purge. No runaway exotherm was observed. Unreacted monomer was distilled off by shutting off the cooling condenser, increasing the heat input to the flask and purging with nitrogen for 4 hours. The resulting hot dispersion of polymer beads was filtered through two layers of cheesecloth, and the beads washed with four 5-liter tap water charges followed by two 3-liter deionized water charges. The beads were then spread on a release-coated paper and dried for two days at 65° C. Gel permeation chromatography was used to determine the weight average molecular weight (356,432) and number average molecular weight (103,529) of the polymer. Differential scanning calorimetry was used to determine the glass transition temperature of the polymer (62.8° C.).

A toner powder was then made in the same way as that of Example 1 except that the starting ingredients were:

|                                              |          |
|----------------------------------------------|----------|
| Magnetite powder (Citco)                     | 60 parts |
| Copolymer of styrene and of isoctyl acrylate | 36       |
| Armeen TM 2HT                                | 4        |
| Raven TM 5750 Carbon black                   | 2        |

The resulting toner powder was tested for transmission image density in the same manner as were the ton-

ers of Examples 1 and 2. The doctor blade gap was 0.46mm, the development gap was 0.5mm, and the developer shell rotated at 350 rpm (development speed of 24 cm/sec). The transmission densities obtained are set out in Table III.

TABLE III

| Voltage | Transmission Density (O.D.U.) |
|---------|-------------------------------|
| -1300   | 1.7                           |
| -1000   | 1.05                          |
| -750    | 0.65                          |
| -500    | 0.15                          |
| -200    | 0.02                          |
| 200     | 0.02                          |
| 500     | 0.02                          |
| 750     | 0.02                          |
| 1000    | 0.05                          |
| 1300    | 0.7                           |

The data indicate that the toner charged inherently strongly positive.

## EXAMPLE 5

The toner powder of this Example was made in the same way as that of Example 2 except that the starting ingredients were:

|                                                    |          |
|----------------------------------------------------|----------|
| Magnetite powder (Citco)                           | 60 parts |
| Styrene/Isooctylacrylate                           | 36       |
| Polymer of Example 4                               |          |
| Amine-containing aliphatic wax adduct of Example 2 | 4        |
| Raven TM 5750 Carbon Black                         | 2        |

The resulting toner powder was tested for transmission image density in the same manner as were the toners of Examples 1 and 2. The doctor blade gap was 0.46mm, the development gap was 0.5mm, and the developer shell rotated at 350 rpm (development speed of 24 cm/sec). The transmission densities obtained are set out in Table IV.

TABLE IV

| Voltage | Transmission Density (O.D.U.) |
|---------|-------------------------------|
| -1300   | 1.65                          |
| -1000   | 1.02                          |
| -750    | 0.65                          |
| -500    | 0.25                          |
| -200    | 0.04                          |
| 200     | 0.02                          |
| 500     | 0.02                          |
| 750     | 0.11                          |
| 1000    | 0.22                          |
| 1300    | 0.6                           |

The data indicate that the toner charged inherently strongly positive.

What is claimed is:

1. Monocomponent toner powder comprising a plurality of discrete particles, each a mixture of (1) a thermoplastic binder comprising at least one copolymer of styrene having a glass-transition temperature ranging from about 45° to about 75° C. and at least one of acrylate and methacrylate monomers and (2) magnetically responsive material, wherein the improvement comprises:
- 5 from 0.5 to 20 percent by weight of the thermoplastic binder is amine-containing aliphatic wax having a secondary amine group adducted with an acrylate, said amine-containing aliphatic wax having two carbon chains of at least 12 carbon atoms each.
- 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 952

UNITED STATES PATENT AND TRADEMARK OFFICE  
CERTIFICATE OF CORRECTION

PATENT NO. : 4,833,056

Page 1 of 2

DATED : MAY 23, 1989

INVENTOR(S) : S. K. BHATEJA, C. I. YOUNG, N. N. QUAN

It is certified that error appears in the above-identified patent and that said Letters Patent is hereby corrected as shown below:

Col. 1, line 35, "electrophotography" should be

— electrophotography —.

Col. 4, line 13, "33" should be — 3 —.

Col. 4, line 17, "(T)" should be — (Tg) —.

Col. 5, line 36 " $(C_{18}H_{37})NH$ " should be —  $(C_{18}H_{37})_2NH$  —.

Col. 7, line 12 "lhe" should be — The —.

Col. 7, line 38 "Curves" should not be in bold print and  
should begin a new paragraph.

Col. 7, line 42 "tone:" should be — toner —.

Col. 9, line 8 "a hot" should be — a = hot —.

Col. 9, line 68 "5" should be — 65 —.

Col. 10, line 2 " $(C_{18}H_{37})_2NH$ " should be —  $(C_{18}H_{37})_2NH$  —.

Col. 12, line 25 after "formula" add —  $(C_{18}H_{37})_2NH$  —.

UNITED STATES PATENT AND TRADEMARK OFFICE  
CERTIFICATE OF CORRECTION

PATENT NO. : 4,833,056

Page 2 of 2

DATED : May 23, 1989

INVENTOR(S) : S. K. Bhateja, et al

It is certified that error appears in the above-identified patent and that said Letters Patent is hereby corrected as shown below:

Column 12, line 27, "I" should be -- 1 --.

Signed and Sealed this  
Twenty-seventh Day of March, 1990

Attest:

JEFFREY M. SAMUELS

Attesting Officer

Acting Commissioner of Patents and Trademarks